

## UNITED STATES PATENT OFFICE

JACOB WOLFSON, OF BROOKLYN, NEW YORK, AND DOROTHY LANGDON POTTER, OF HACKENSACK, NEW JERSEY, ASSIGNEES TO NATIONAL OIL PRODUCTS COMPANY, OF HARRISON, NEW JERSEY, A CORPORATION OF NEW JERSEY

## PROCESS FOR THE TREATMENT OF TEXTILE FIBERS

No Drawing.

Application filed July 31, 1929. Serial No. 382,582.

Our invention relates to a process for the treatment of textile fibers and relates particularly to a process adapted for the treatment of silk.

5 In the preparation of silk it is essential that the waxes and gums be softened and that it be converted into a soft, pliable condition and for certain uses, as for hosiery tram, it is desirable that the silk be hygroscopic in order that it may be knitted direct from the cone without the necessity of back winding, which requires an additional softening treatment.

10 This softening of the silk fiber and gum has usually been accomplished by immersing the fiber in a bath of water and emulsified oil for about 12 hours, removing and whizzing. This process allows a large amount of oil to remain in the bath, thus causing a loss 15 thereof, the fibers are not uniformly penetrated and are not hygroscopic. Attempts have been made to introduce electrolytes into the treatment bath but many of these have a tendency to break the emulsion and hence 20 are useless for the intended purpose.

Our process overcomes the above-mentioned, and other, objectionable features of the present employed methods for the treatment 25 of silk and presents a method whereby emulsification is retained, the gums and waxes are softened, a practical exhaustion of all of the oil by the silk is obtained, better penetration is accomplished, a more uniform result is obtained and the treated silk is hygroscopic and can be knit without back winding.

30 The process of our invention comprises introducing an aromatic hydroxy compound, a salt of a sulpho acid of an aromatic hydroxy compound or a derivation thereof into the treatment bath, among which are a salt of beta naphthol 3:6 disulpho acid (R acid), a salt of beta naphthol 6 monosulpho acid (Schaffer's acid), a salt of alpha naphthol 4 monosulpho acid (N. W. acid), a salt of 35 sulphonated cresol.

We give the following as one example of our process:

An emulsion is made of 14 pounds soluble olive oil (sulphonated olive oil) and 40 gallons of water.

2 pounds of R salt are dissolved in 40 gallons of water.

The emulsion is added to, and thoroughly mixed with, the solution of R salt and 100 pounds of silk are immersed therein for 12 55 hours, removed and whizzed.

By our process practically all of the soluble oil is absorbed by the silk from the bath, whereas in the present employed process about 18 pounds of oil would be employed, 60 only about 20 percent of which is absorbed, the remainder being wasted.

In addition to this economic advantage, our process produced better and more even penetration and makes the silk hygroscopic, all 65 of which qualities are of the greatest advantage in the further treatment of the fiber.

By "aromatic hydroxy compounds" in our claims we mean the aromatic hydroxy compounds themselves, their salts, their sulpho 70 acids and derivations, whether used singly or in combination with each other.

We do not limit ourselves to the particular chemicals, time of treatment, or steps of procedure specifically mentioned, as these are 75 given simply as a means for describing the process of our invention.

What we claim is:—

1. In the treatment of textile fibers, the step which comprises treating the fiber with 80 a soluble oil and an aqueous soluble salt of beta naphthol 3:6 disulpho acid.

2. In the treatment of textile fibers, the step which comprises treating the fiber with soluble olive oil and an aqueous soluble salt 85 of beta naphthol 3:6 disulpho acid.

3. In the treatment of silk, the step which comprises treating the fiber with a soluble oil and an aqueous soluble salt of beta naphthol 90 3:6 disulpho acid.

4. In the treatment of silk, the step which comprises treating the fiber with soluble olive oil and an aqueous soluble salt of beta naphthol 3:6 disulpho acid.

5. In the treatment of textile fibers, the step which comprises treating the fiber with a soluble mineral oil and an aqueous soluble salt of beta naphthol 3:6 disulpho acid.

6. In the treatment of silk, the step which 100 comprises treating the fiber with a soluble

mineral oil and an aqueous soluble salt of beta naphthol 3:6 disulpho acid.

7. In the treatment of textile fiber, the step which comprises treating the fiber with a soluble oil and an aqueous soluble salt of a sulpho acid of an aromatic hydroxy compound.

8. In the treatment of textile fiber, the step which comprises treating the fiber with a soluble olive oil and an aqueous soluble salt of a sulpho acid of an aromatic hydroxy compound.

9. In the treatment of silk fiber, the step which comprises treating the fiber with a soluble oil and an aqueous soluble salt of a sulpho acid of an aromatic hydroxy compound.

10. In the treatment of silk fiber, the step which comprises treating the fiber with a soluble olive oil and an aqueous soluble salt of a sulpho acid of an aromatic hydroxy compound.

11. In the treatment of textile fiber, the step which comprises treating the fiber with a soluble mineral oil and an aqueous soluble salt of a sulpho acid of an aromatic hydroxy compound.

12. In the treatment of silk fiber, the step which comprises treating the fiber with a soluble mineral oil and an aqueous soluble salt of a sulpho acid of an aromatic hydroxy compound.

13. In the treatment of textile fiber, the step which comprises treating the fiber with soluble mineral oil and an aqueous soluble salt of beta naphthol 3:6 disulpho acid.

Signed at Harrison, in the county of Hudson and State of New Jersey, this 25th day of July, 1929.

JACOB WOLFSON.  
DOROTHY LANGDON POTTER.